

## UNITED STATES PATENT OFFICE

2,459,119

## CORROSION RETARDER

John T. Rucker, Lewiston, N. Y., assignor to  
 Hooker Electrochemical Company, Niagara  
 Falls, N. Y., a corporation of New York

No Drawing. Application September 27, 1946,  
 Serial No. 699,640

3 Claims. (Cl. 252—148)

1

My invention relates more particularly to retarders of corrosion of metals by acids.

It is known that certain substances exert a protective effect upon metals, against attack of acids thereon, by rendering the metal passive with respect to the acid, i. e., as anti-catalysts. I will refer to these hereinafter as "inhibitors." It is also known that certain other substances exert a protective effect by interposing a film between the metal and the acid. These are of the nature of detergents, or dispersing or wetting agents, characterized by low surface tension. I will refer to these hereinafter as "surface active" materials.

Among the agents of the inhibitor category are the aralkyl thio-cyanates, such as benzyl and cymene thiocyanates. These are typical examples of aralkyl thio-cyanates, each having a methyl group, to which the thio-cyanate group is attached, and the cymene having, in addition, a propyl group. However, these compounds are of low solubility in acid pickling baths. Also, benzyl thio-cyanate has not only an exceedingly disagreeable odor, but toxic and lachrymatory properties, the effects of which are aggravated by its low solubility and consequent tendency to collect at the surface of the bath and spatter into the atmosphere. For these reasons, these compounds have heretofore had little importance, except under conditions permitting of vigorous agitation.

Among the agents of the surface active category are the quaternary ammonium compounds, such as lauryl pyridinium chloride and lauryl dimethyl benzyl ammonium chloride. These are selected examples of quaternary ammonium compounds in which the nitrogen is in the ring and chain respectively. They are not only quite soluble in acid pickling baths, but also have the property of increasing the solubility of other organic compounds, including the thio-cyanates. When used in pickling baths, their saponaceous character causes them to form a foam layer upon the surface.

The effectiveness of these surface active materials is illustrated by the following examples, in which the abbreviations "LPC" and "LDBAC" stand for lauryl pyridinium chloride and lauryl dimethyl benzyl ammonium chloride respectively, and the expression "protection, per cent" signifies the extent to which the agent is effective in eliminating corrosion altogether:

## Example I

|                              |       |          |        |        |
|------------------------------|-------|----------|--------|--------|
| Metal, steel                 |       |          |        |        |
| Acid, sulphuric, 25%         |       |          |        |        |
| Temperature, 20° C.          |       |          |        |        |
| Corrosion retarder.....      | None  | LPC      | LPC    | LDBAC  |
| Per cent retarder by wt..... |       | 0.1      | .02    | 0.1    |
| Wt. loss p. sq. c. m.        |       |          |        |        |
| p. hr., g.....               | .0034 | .0000057 | .00019 | .00011 |
| Protection, per cent.....    |       | 99.84    | 94.4   | 96.7   |

2

## Example II

|                              |       |        |        |        |
|------------------------------|-------|--------|--------|--------|
| Metal, steel                 |       |        |        |        |
| Acid, hydrochloric, 20%      |       |        |        |        |
| Temperature, 20° C.          |       |        |        |        |
| Corrosion retarder.....      | None  | LPC    | LPC    | LDBAC  |
| Per cent retarder by wt..... |       | 0.1    | .02    | 0.1    |
| Wt. loss p. sq. c. m.        |       |        |        |        |
| p. hr., g.....               | .0043 | .00012 | .00025 | .00015 |
| Protection, per cent.....    |       | 97.2   | 94.3   | 96.4   |

## Example III

|                              |      |       |      |       |
|------------------------------|------|-------|------|-------|
| 10 Metal, steel              |      |       |      |       |
| Acid, sulphuric, 15%         |      |       |      |       |
| Temperature, 75° C.          |      |       |      |       |
| Corrosion retarder.....      | None | LPC   | LPC  | LDBAC |
| Per cent retarder by wt..... |      | 0.1   | .02  | 0.1   |
| Wt. loss p. sq. c. m.        |      |       |      |       |
| p. hr., g.....               | .119 | .0022 | .048 | .0016 |
| Protection, per cent.....    |      | 98.2  | 60.0 | 98.7  |

It will be seen from the above examples that the addition of minute quantities of these materials to acid pickling baths greatly diminishes the attack upon steel.

15 The effectiveness of the aralkyl thio-cyanates, with vigorous agitation, is illustrated by the following example, in which "BTC" and "CTC" stand for benzyl and cymene thio-cyanates respectively:

## Example IV

|                                       |  |  |      |       |
|---------------------------------------|--|--|------|-------|
| Metal, steel                          |  |  |      |       |
| Acid, sulphuric 15%                   |  |  |      |       |
| Temperature, 75° C.                   |  |  |      |       |
| Corrosion retarder.....               |  |  | None | BTC   |
| Per cent retarder by wt.....          |  |  | .02  | CTC   |
| Wt. Loss per sq. c. m. p. hr., g..... |  |  | .119 | .0010 |
| Protection, per cent.....             |  |  | 99.2 | 99.2  |

Lauryl pyridinium chloride and lauryl dimethyl benzyl ammonium chloride are partially soluble in oils. They are water soluble and also quite soluble in oils. I have now found that, when these compounds are used in combination with benzyl or cymene thio-cyanates they act as dispersing agents for the thio-cyanates, besides increasing their solubility. Moreover, the foam layer formed by the surface active agents suppresses the tendency of the thio-cyanate to spatter and renders its use unobjectionable. In substantially equal proportions by weight lauryl pyridinium chloride forms with benzyl thio-cyanate a eutectic melting at 15° C. In the same proportions it forms with cymene thio-cyanate a composition that is liquid at room temperature. I have found these compositions to be exceptional corrosion retarders.

45 This is illustrated by the following example:

## Example V

|                                      |  |       |      |         |
|--------------------------------------|--|-------|------|---------|
| 55 Metal, steel                      |  |       |      |         |
| Acid, sulphuric, 15%                 |  |       |      |         |
| Temperature, 75° C.                  |  |       |      |         |
| Corrosion retarder.....              |  | LDBAC | 50%  | LPC 50% |
| Per cent retarder by wt.....         |  | BTC   | 50%  | CTC 50% |
| Wt. loss p. sq. c. m. p. hr., g..... |  | .02   | .02  | .02     |
| Protection, per cent.....            |  | .0011 | .001 | .00076  |

It will be seen by comparison of Example V with Examples III and IV that these compositions

are extremely effective. They are not in every case more effective than thio-cyanate by itself, but it must be remembered that these compositions are entirely practicable, whereas the thio-cyanates are generally impracticable. However, the LPC-BTC eutectic is more effective than either of its constituents.

When added to acid pickling baths, these corrosion retarders have in general a selective protective effect upon the metal, as compared with its oxide. This is illustrated by the following:

*Example VI*

|                                              |                              |
|----------------------------------------------|------------------------------|
| Metal, steel, heavily coated with brown rust |                              |
| Acid, sulphuric, 15%                         |                              |
| Temperature, 75° C.                          |                              |
| Corrosion retarder                           | None      LPC 50%<br>BTC 50% |
| Per cent retarder                            | 0.1                          |
| Time of cleaning, minutes                    | 3.0      3.5                 |

*Example VII*

|                                             |                              |
|---------------------------------------------|------------------------------|
| Metal, steel heavily coated with blue scale |                              |
| Acid, sulphuric, 15%                        |                              |
| Temperature, 75° C.                         |                              |
| Corrosion retarder                          | None      LPC 50%<br>BTC 50% |
| Per cent retarder                           | 0.1                          |
| Time of cleaning, minutes                   | 0.5      0.7                 |

It will be seen from Examples VI and VII that the addition of a relatively large quantity of one of my preferred corrosion retarders to the pickling bath increased the time of pickling only very slightly.

In order to show that my corrosion retarders have exceptional properties, I present herewith a table showing the percentage of protection afforded to ferrous metals by a considerable number of the best known corrosion retarders, against 4 per cent sulphuric acid at 71° C. This table is taken from "Chemical Industries," 1935, vol. 37, page 124. The first part of this table is a comparison of certain retarders on the basis of an equal percentage by weight. The second part is a comparison of certain other retarders on the basis of an equal molecular percentage. To each part I have added lauryl pyridinium chloride, lauryl pyridinium thio-cyanate and my LPC-CTC and LPC-BTC compositions, on the appropriate basis.

| Retarder                                        | Mols Per Liter | Wt. Per Cent | Protection Per Cent |
|-------------------------------------------------|----------------|--------------|---------------------|
| Sulfonated oil                                  |                | 0.1          | 10                  |
| Nitrogen base oil                               |                | 0.1          | 30                  |
| Paper waste liquor                              |                | 0.1          | 33                  |
| Sulfonated animal matter                        |                | 0.1          | 63                  |
| Low grade wheat flour                           |                | 0.1          | 85                  |
| Nitrogen bases                                  |                | 0.1          | 88                  |
| Coal Tar nitrogen bases                         |                | 0.1          | 95                  |
| Lauryl pyridinium chloride                      |                | 0.1          | 85                  |
| LPC-CTC                                         |                | 0.1          | 99.4                |
| LPC-BTC eutectic                                |                | 0.1          | 99.99               |
| Triethylamine                                   | .01            | .15          | 10.5                |
| Aniline                                         | .01            | .09          | 14.5                |
| Pyridine                                        | .01            | .08          | 19.0                |
| Quinoline                                       | .01            | .13          | 49.4                |
| Acridine                                        | .01            | .18          | 82.4                |
| 2-me-quinoline                                  | .01            | .15          | 53.0                |
| me-acridine                                     | .01            | .20          | 81.8                |
| Phenyl acridine                                 | .01            | .20          | 90.2                |
| Dimethyl-diethyl-diamino acridine hydrochloride | .01            | .33          | 99.8                |
| Lauryl pyridinium chloride                      | .01            | .20          | 81.8                |
| LPC-CTC                                         | .01            | .25          | 99.5                |
| LPC-BTC eutectic                                | .01            | .22          | 99.99+              |

It will be seen from the above that lauryl pyridinium chloride and lauryl pyridinium thio-cyanate rank high among corrosion retarders, and when it is remembered that they have the advantage over most of them of high water solubility and freedom from offensive odor their importance

as corrosion retarders will be manifest. It will also be seen that my LPC-BTC eutectic tops all of the list, since in equal weight or molecular proportion it has a higher protective value, and for a given protective value much less of it need be used. It should be noted that while the difference between protective values of 99.8 and 99.99+ is not mathematically great, its significance is enormously important, for it means that in the latter case the corrosion rate is less than one twentieth. In other words, steel subjected to 10 per cent sulphuric acid at 71° C. will last more than twenty-times as long if protected by my eutectic as if protected by the best of the previously known corrosion retarders.

Corrosion retarders are useful wherever acids are handled in metal equipment, of which pickling of metal is only one of many illustrations, acid treatment of oil wells being another. Another 20 use for such retarders is in lubricants, which are liable to develop acidity through oxidation, by contact with the air. Organic acids developed in lubricating oils, such as those used in automotive crank cases, are mild compared with pickling acids, but the time factor is measured in months instead of hours, and in the long run the corrosive effect of such acids may be very serious, especially upon bearing alloys, such as those composed of lead, tin, copper and less common metals. It 25 is difficult to give a quantitative measure of the effect of corrosion retarders in lubricating oils, as the matter is complicated by wear. Nevertheless, visual comparison of the effects of lubricating oils upon bearings, with and without my retarders, indicates that my retarders have a 30 useful effect in such oils.

While I have given examples of the results obtained with my compositions only in equal proportions by weight, I do not wish to be limited to 40 such proportions, as any small addition, such as 10 per cent, of these and other analogous aralkyl thio-cyanates, of low solubility, to the quaternary ammonium compounds mentioned and other analogous compounds, of good solubility 45 and having the property of dispersing, and increasing the solubility of, the thio-cyanate, will improve the corrosion retarding properties of the quaternary ammonium compounds, and the addition of as little as 20 per cent of the latter to the thio-cyanate is useful in suppressing its spattering tendency. Also, while in the examples the proportion of corrosion retarder ranges from 0.02 to 0.1 per cent by weight, I do not wish to be held to these limits, as my retarders are useful in proportions as low as .005 per cent, and there is no objection to using up to 5 per cent of the retarder.

In the foregoing examples I have given tests only of compositions of benzyl and cymene thiocyanates with lauryl pyridinium chloride and lauryl dimethyl benzyl ammonium chloride, but these 50 are given as typical only. Besides these, many combinations of other aralkyl thio-cyanates, such as xylyl thio-cyanate, and mesityl thio-cyanate, etc., with other quaternary ammonium compounds, such as lauryl pyridinium sulphonate, trimethyl cetyl ammonium chloride, amido benzyl pyridinium chloride, etc., form compositions 55 which are superior retarders of corrosion of metals by acids. In short, any aralkyl thiocyanate 60 in combination with a quaternary ammonium compound, and in particular those having an acid radical and an alkyl group of at least 10 carbon atoms attached to the nitrogen atom, the remaining nitrogen valences being satisfied by 65 carbon members of one or more hydrocarbon rad-

icals, one of which may be benzyl and the others of which may be methyl, or which may be a five membered heterocyclic carbon ring, or any quaternary ammonium thio-cyanate, comes within the scope of my invention.

I claim as my invention:

1. As a new composition of matter, useful as a retarder of corrosion of metals by acids, a substantially eutectic mixture consisting of lauryl pyridinium chloride and benzyl thiocyanate in substantially equal proportions by weight.

2. The method of eliminating at least 99.99 per cent of the corrosion of ferrous metals by acid pickling baths, such as 4 per cent sulphuric acid at 71° C., which comprises incorporating in the acid substantially 0.1 per cent of its weight of a substantially eutectic mixture consisting of lauryl pyridinium chloride and benzyl thiocyanate.

3. The method of protecting bearing metals in

automobile crankcases against organic acids developed in lubricating oils during use therein, which comprises incorporating in the oil 0.005 to 0.1 per cent of a substantially eutectic mixture of lauryl pyridinium chloride and benzyl thiocyanate.

JOHN T. RUCKER.

#### REFERENCES CITED

The following references are of record in the file of this patent:

#### UNITED STATES PATENTS

| 15 | Number    | Name                 | Date           |
|----|-----------|----------------------|----------------|
|    | 2,006,216 | MacArthur et al. --- | June 25, 1935  |
|    | 2,016,035 | Downing et al. ----- | Oct. 1, 1935   |
|    | 2,203,649 | Felkers -----        | June 4, 1940   |
|    | 2,296,433 | Frey et al. -----    | Sept. 22, 1942 |